

## UNITED STATES PATENT OFFICE

RICHARD PAUL CARLTON, OF ST. PAUL, MINNESOTA, ASSIGNOR TO MINNESOTA MINING AND MANUFACTURING COMPANY, OF ST. PAUL, MINNESOTA, A CORPORATION OF MINNESOTA

## COMPOSITE STRUCTURE

No Drawing. Application filed December 29, 1923, Serial No. 683,523. Renewed June 28, 1927.

This invention relates to abrasives and the like and more particularly to moisture-proof flexible abrasive devices, and more especially with reference to improvements in moisture-proof, that is, water, oil and other wet proof abrasive material which is characterized by tenacity and, preferably, flexibility, and which is capable of use in the presence of dampness or wetness without immediate disintegration due thereto, and specifically to so-called cellulosic binders.

It will be understood by those skilled in the art that cellulosic material disclosed as employed by me is intended to include such 15 cellulosic material, treated or otherwise, which may be suitable for employment in this connection, such for example, as cellulose nitrate, cellulose acetate and cellulose xanthogenate.

20 This invention is characterized as employing cellulose as one of its principal ingredients, in combination, where necessary, as will hereinafter appear, with a modifying agent for increasing the adhesive properties of the 25 cellulose and as well enhancing the strength thereof without interfering with or reducing its flexibility where desired, and while a specific modifying agent or agents are mentioned as this description proceeds, and while 30 the invention is described for use as a moisture-proof binder for sandpaper or other abrasive devices, fabric or otherwise, it will be understood that they are set forth as illustrations of the employment of a particular in- 35 gredient or ingredients or proportions of such ingredients for my present purposes, and that the field of utility of the binder and the abrasive device is of wide application:

30 This invention has as one of its principal 40 objects the employment of cellulosic material, such as cellulose nitrate, cellulose acetate, et cetera, as the basis for an improved binder for securing pulverulent or com- 45 minuted abrasive material to a flexible back- 50 ing formed either of similar material as that of the binder or a derivative thereof, or formed of paper, cloth, or other suitable fabric, and this invention contemplates the use of a backing which may or may not be 55 waterproof or moisture-proof per se or of a

backing which may or may not be first rendered moisture-proof before receiving the binder and the abrasive. I contemplate the employment of my invention for one or more of the following purposes, viz: as an improved binder per se, and as a binder on paper or cloth which has previously been rendered moisture-proof, such as by oil saturation, varnish, moisture-proof glue, or the like, or by the employment of the ma- 55 terial of this invention as a moisture proofing material for a backing.

50 My practice hereinafter described which has resulted in the production of a moisture-proof, highly tenacious and flexible abrasive 55 sheet, has been carried on with cellulose in various forms, and various solutions and modifications. With the object in mind of producing the product in large quantities at a reasonable cost, I have employed among 60 other things, the various nitro-cellulose products, including so-called leather solutions and those commonly known as powder dopes, made by converting powder, of which latter 65 there were large stocks remaining as surplus 70 material after the recent "great war". This power dope, so-called, when reduced, affords a cellulose nitrate solution of low fiber content and as a bond for moisture-proof abrasive devices is capable of being rendered prac- 75 ticable if modified as hereinafter pointed out. The cellulose materials are generally classified according to their content of fiber and it 80 will readily be understood that the better cellulose solutions contain a greater quantity 85 of fiber and therefore a better body is imparted to the material. I do not reject the higher fiber content cellulose solutions, but I have found that by my invention I am enabled 90 to use the cheaper grades by combining there- 95 with in suitable proportions a modifying agent which is in itself moisture-proof, flexible and tenacious for imparting to the cheaper grade of cellulose suitable body, tenacity, and adhesive quality without detracting 95 from the flexibility of the product when set. I have found that where cellulose is employed as a binder when applied with a suitable abrasive, to celluloid, the adhesiveness of the 100 binder is materially increased as well as the

tenacity if a modifying agent is employed, and this is particularly true of the lower grades of cellulose or its derivatives. For this reason, and others to appear, I have employed cellulose in combination with a modifying agent such as resin, either natural resin or synthetic resin. This invention also has a principal object thereof the employment of cellulose or the like and a modifying agent 5 as a binder for attaching comminuted abrasive material to a sheet of fabric or the like. Therefore, the principal objects and advantages of this invention reside in the provision of an improved moisture-proof binder including cellulose material; the provision of an improved flexible moisture-proof binder including cellulose material and a modifying agent; the provision of an improved binder, including cellulose material, for attaching 10 grit to paper sheets or cloth or fabric; and the provision of an improved binder characterized by flexibility, tenacity, and imperviousness to moisture which includes cellulose material and a modifying agent, for 15 the purpose of increasing the tenacity of the binder without reducing the flexibility or durability thereof.

As I have hereinbefore mentioned, the cellulose product known as powder dope, due 20 to its low fiber content, for the purposes of this invention, requires a modifying agent or filler, and I have discovered that either certain natural or synthetic resins combined with the cellulose material and with a suitable 25 solvent produces a binder which is moisture-proof and is possessed of a high degree of tenacity and will readily combine with paper, cloth or a suitable base formed of the same or a similar material, such as celluloid, 30 and will be more efficacious for the purposes contemplated than a binder not containing such a modifying agent.

Certain cellulose solutions produced from powder are in some cases very explosive and 35 others are not of an explosive nature. They may be classified as cellulose mononitrate which contains a percentage of nitrogen to about 7 percent; cellulose dinitrate containing 40 11 to 12 percent nitrogen; and cellulose trinitrate containing from 14 to 14.15 percent 45 nitrogen. I find that all these classes are readily soluble in suitable solvents and are suitable for the purpose of this invention, though some of them would preferably require 50 conversion to bring the high nitrates into a lower nitrate, such as by boiling with dilute nitric acid, thereby preventing explosion 55 either in manufacture or use.

The above classification of the cellulose 60 solutions merely serves to indicate these products as they are produced in their crude state, the finished product now obtainable in the open market being a solution of these solid cellulose materials. The quantity of the 65 solid which is taken up by the solvent deter-

mines the fiber content of the cellulosic solution. A solution wherein the fiber content is about 50 to 55 percent is now readily obtainable. This is called a 70 ounce solution, that is 70 ounces of the solid are taken up per gallon of the aggregate. It will be obvious to 70 those skilled in the art that the higher the percentage of fiber content, the tougher the film and therefore the more the substance becomes desirable for use as a binder such as for sandpaper.

The usual solvents for nitro cellulose are amyl acetate, amyl alcohol, butyl alcohol, acetone and ether alcohol mixtures. There are a large number of cellulose solutions now in the market and as solvents thereof amyl acetate or amyl alcohol in combination with benzene (benzol) or fusel oil may be employed, the fusel oil and benzene (benzol) serving as 80 thinners. In these cellulose solutions the solvents mentioned above are preferred because the resultant films are clear as distinguished from the result obtained when solvent with hygroscopic tendencies such as acetone is employed, due to the tendency of such solvents 85 to absorb water from the air. It is therefore obvious that to make a moisture-proof binder it is preferable that the cellulosic solution be treated by either amyl acetate, amyl alcohol or other non-hygroscopic solvent so as to prevent any absorption of moisture as explained.

I have, in the course of my practice, employed nitro cellulose varnishes, a particular one, for example, having a fiber content of approximately 30 percent of the solution, gum camphor being preferably a constituent of this varnish because it acts to materially reduce the inflammability thereof or the tendency of the solution to explode. Flexibility is imparted to the film produced by adding castor oil in small percentages, usually below 10 percent.

In addition to these materials, that is, gum camphor and castor oil, I have further modified the cellulosic solution by the addition thereto of gums such as shellac, kauri, dammar, pontianak, cumoron, and either natural or synthetic resins.

In my practice I have employed gum pontianak in quantity about 10 percent by weight 115 to a quantity of cellulose varnish and good results are obtained. Any of the gums mentioned hereinbefore are readily soluble directly in the varnish since the amyl acetate used as a solvent for the cellulose nitrate is also a 120 rapid solvent for the gum.

Under ordinary conditions the addition of any of the above mentioned gums to the higher fiber content cellulose varnish is not so absolutely necessary as the addition of such 125 gums to the cheaper cellulosic materials, such as that known as powder dope, but at all times materially improves the appearance, body and tenacity of the binder without interfering with the flexibility desired where the binder 130

is applied to a flexible sheet. The cheaper cellulose dopes commercially available are usually dissolved in low boiling point alcohols and give an insufficient body for supporting the abrasive material, but the gums added to the cellulosic material retain their adhesive nature after the cellulosic film has had surface coagulation and thus improve the aggregate as a binder.

10 In the employment of cellulosic solutions wherein the fiber content is high, amyl acetate or amyl alcohol is employed by me as the solvent as this material dries comparatively slowly which makes it possible for the 15 minuted abrasive to penetrate the film applied to the paper or fabric before the same has had surface coagulation.

From the foregoing it will be seen that in the case of cheaper dopes it is necessary to 20 modify the cellulosic solution in order to permit of application of the abrasive substance before the film of adhesive congeals, and that in the case of the more expensive dopes I 25 utilize a solvent having desired predetermined qualities.

In manufacturing an abrasive sheet in accordance with this invention, and assuming that the cheaper dopes are employed in the binder, it will be understood from the 30 foregoing that any of the gums hereinbefore mentioned may be combined with the cellulosic solution for two purposes at least, the principal purpose being to increase the tenacity of the solution and the binder, and 35 secondly to retard the drying sufficiently to permit of introduction of the abrasive material into the binder before coagulation or skinning over has set in. The addition of either the natural or synthetic resins will 40 accomplish this result very nicely and one example of a practicable application of this invention as to proportions employed is as follows:

10 parts 30 oz. cellulose nitrate solution, 45  $\frac{3}{4}$  part gum pontianak added directly to above solution,  $\frac{1}{4}$  part gun camphor,  $\frac{1}{2}$  part castor oil.

In the practice of my invention I find that success is obtained in the employment 50 of a plasticizer, such as gum camphor, and I also find that for certain purposes the combination of an acetate, a ketone, such as acetone, benzol, and plasticizer and a gum such as gum pontianak combined with the 55 cellulose nitrate solution gives desirable results.

In order to get a form of nitro-cellulose which can be used in solution and possess properties essential for operation on a production basis, such as even flowing or spreading on the backing used, there must be a certain balance of high, medium and low boiling solvents to obtain the proper rate of evaporation. To get the gum, like 65 dammar, into solution, and the nitro-cellulose

into solution, the lower boiling solvents, such as ethyl alcohol, acetone and an acetate are used. To prevent too rapid evaporation and thus provide for the proper flow of the material, additional solvents of relatively higher boiling points, such as butyl, and amyl acetates, the higher boiling alcohols, and certain ketones are used. Low evaporation rate, produced by higher boiling solvents prevents cooling of the surrounding air and the consequent condensation of water on the lacquer surface. This in turn prevents precipitation of the nitro-cellulose. Thus the important adjustment of the solution to the proper boiling point is secured.

Benzol is used as a diluent and also as a solvent for the gums used because of its comparatively low cost. It functions to reduce the viscosity of the nitro-cellulose solution containing gums so that it is easier to manipulate in the abrasive coating process.

Camphor, castor oil, phosphates, such, for example, as tri-cresol phosphates; tartrates, such as butyl tartrates, phthalates such as dibutyl phthalate have all been successfully employed by me and form excellent plasticizers or softeners. The function of such a plasticizer or softener is to make the resulting film tough, elastic, flexible, adhesive 30 and permanent.

The function of the gum is to give adhesion, body and hardness to the coating and to render the coating more impervious to moisture. This increase in the hardness of the film is a very desirable feature in producing a good abrasive paper because the abrasive grains on the paper undergo very severe service in the art of rubbing or grinding the materials on which they are being 40 worked, and by increasing the hardness of the film the grains are more firmly held in place and stick on to the backing longer and more securely so that the life of the abrasive article is increased. The gum also increases the body of the coating material without increasing the viscosity thereof, and this is highly desirable. Being cheaper than nitro-cellulose, many gums tend to reduce the cost. In increasing the hardness 50 by the use of a gum there is a tendency to brittleness, and to offset this and secure plasticity is one of the functions of the plasticizer, such as camphor.

I find that I am enabled to produce a successful waterproof abrasive product with the usual backing incorporating thereon a film formed by evaporation from a modified nitro-cellulose composition including a low boiling solvent, such as other alcohol mixtures, a high boiling solvent, such as amyl acetate, for retarding the evaporation, and a gum acting as an element for giving body to the composition, that is, in the nature of a filler, benzol, and a plasticizer. Therefore, 65

to this end the waterproofing substance may be proxylyn dissolved in a proper solvent, such as an acetate, with or without other acetates such as ethyl alcohol, and with or without other alcohols, ketones like acetone, methyl ketones or acetone oils, benzol and camphor.

I also contemplate applying the binder of this invention to a base layer or member which is formed of material of the same nature, such as applying the cellulose binder to a celluloid sheet or strip or disc (the arrangement in such a case preferably including first the celluloid sheet, secondly a coating of my improved binder, then a coating of the same binder containing grit applied thereto, and lastly a sizing coating. In this manner the continuity of the base layer is not disturbed by the grit and the base layer thus retains its original strength.

I also contemplate employing this invention in connection with oiled paper or with any other paper or fabric which has previously been rendered waterproof or moisture-proof by impregnation or partial impregnation or by applying a coating of waterproof material to the back thereof. Such waterproofing material may be my present binder suitably thinned.

30 After the product is set, I apply a sizing coat or coats which may be of the same solution as that used for carrying the grit but generally without thinning it, though, of course, where a very heavy body solution such as those referred to hereinbefore is employed it is necessary to thin such a solution to a sufficient extent to facilitate its handling and any of the solvents mentioned hereinbefore may be employed for this purpose.

40 Again, especially in employing the cheaper dopes, such as cellulose solutions having a small fiber content, it is desirable that when applied to paper, the latter be sized to improve the bond between the base and the adhesive, and to prevent the base or making coat from penetrating too greatly, so that this making coat of the binder will not be unduly reduced in strength but will be thick enough to receive the abrasive substance.

50 The application of a sizing coat to the base may be followed advantageously, even with the higher fiber content cellulose solutions.

There is a considerable quantity of cellulose dopes of other kinds manufactured and in the market today and produced similarly to cellulose nitrate, such for example as cellulose acetate and cellulose xanthogenate. These cellulose dopes are usually non-inflammable and have much the same characteristics and properties as cellulose nitrates but are as a rule more viscous and therefore more difficult to handle in manufacturing. I have carried on practice with such cellulose dopes, and while satisfactory rough results are obtainable, in cases of these solutions and other

solutions of low fiber content it is desirable that repeated layers of the solutions be applied to produce a composite film so as to attain the desired penetration, thickness and strength and tenacity, whether for the binding coat or for the sizing coats.

70 In the production of cellulose acetate dope, cotton fiber, for example, may be subjected to the action of acetic anhydrid, and the resultant solid cellulose acetate dissolved in suitable solvents, such as nitrobenzol, chloroform, etc. In the production of cellulose xanthogenate, the cellulose may be subjected to the action of caustic soda, and then dissolved in suitable solvents such as carbon bisulphide.

75 The following formula is suggested for a cellulose acetate solution applicable as a bond for sandpaper:

80 10 parts saturated solution cellulose acetate in acetone, 1 part shellac gum,  $\frac{3}{4}$  parts castor oil.

85 The following formula is suggested for the production of cellulose xanthogenate but is only a making process for this substance:

90 2 parts cotton fiber, 30 parts 15% caustic soda solution. Steep for 24 to 36 hours. Add 1 part carbon bisulphide. Stir from time to time until dissolved. Thin to a working consistency with water or additional carbon bisulphide.

95 Having thus described my invention and illustrated its use, what I claim as new and desire to secure by Letters Patent is:

1. A flexible abrasive device comprising a plurality of moisture-proof layers of cellulosic material united to form a substantially homogeneous piece, a flexible modifying agent for said layers for imparting increased strength and adhesiveness thereto, and abrasive material embedded in one of said layers.

100 2. A flexible abrasive device for employment in a water-abrading operation comprising a plurality of moisture-proof layers intimately united to form a substantially homogeneous piece, a modifying agent embodied in one of said layers, a moisture-proof flexible base for said layers which is continuous and unbroken and abrasive material embedded in one of said layers.

105 3. An abrasive article comprising a moisture-proof flexible body layer having a grit-carrying coating of moisture-proof flexible stable material and having a modifying agent therein for increasing its tensile strength, and to render the same stable and waterproof when used in a water abrading operation intimately combined therewith to form a substantially homogeneous moisture-proof piece, the grit being carried by said coating.

110 4. A flexible abrasive device comprising a plurality of moisture-proof layers intimately united to form a substantially homogeneous piece, a modifying agent embodied in one of said layers, the base layer being continuous

125

130

135

140

145

150

155

160

165

170

175

and unbroken to impart strength to the device, and abrasive material embedded in one of said layers.

5. A flexible abrasive device comprising a moisture-proof layer, said layer having one of its surfaces provided with grit united thereto by a cellulose cement containing a modifying agent.

10. A flexible abrasive device comprising a moisture-proof layer of flexible material containing a modifying agent, said layer having one of its surfaces provided with grit united thereto by a cellulose cement containing a modifying agent.

15. An abrasive device comprising a moisture-proof base layer provided with a coating of a material having a modifying agent therein, said coating having one of its surfaces provided with grit united thereto by a cellulose cement which is a partial solvent 20 of the material of said coating.

25. An abrasive device comprising a moisture-proof base layer provided with a coating of a material having a modifying agent therein, said coating having one of its surfaces provided with grit united thereto by a cellulose cement containing a modifying agent and which cement is a partial solvent 30 of the material of the base layer.

35. An abrasive article comprising a moisture-proof flexible body layer of cellulosic material, having a modifying agent therein for increasing its tenacity, and having a grit-carrying coating of moisture-proof flexible material intimately combined therewith, and said coating having a modifying agent to 40 form a substantially homogeneous moisture-proof piece, the grit being carried by said coating.

45. An abrasive article comprising a moisture-proof flexible body layer having a modifying agent therein for increasing its tenacity and having a grit-carrying coating of moisture-proof flexible material having a modifying agent and intimately combined with the base layer to form a substantially homogeneous moisture-proof piece, the grit being carried by said coating, whereby the original strength of the body layer is not 50 affected by the grit and the device is capable of continued use wet or dry until the grit is worn away.

55. The method of making abrasive sheets, which includes the step of applying thereto a binder containing cellulosic material and a modifying agent for the cellulose.

60. The method of making abrasive sheets, which includes the step of applying thereto a binder containing a material which is a partial solvent of the material of the sheet, and increasing the bond between the adhesive and the sheet by the provision of a modifying agent in said binder.

65. The method of making a flexible abrasive article for use in a water abrading oper-

ation which includes applying to a flexible sheet of fabric a grit or layer of abrasive particles, and a waterproof bond containing cellulosic material of a nature to maintain the bonding effect throughout the effective abrading life of the abrasive article when employed in a water abrading operation, and applying thereto a plurality of auxiliary coats.

70. The method of making a flexible abrasive article for use in a water abrading operation which includes applying to a flexible sheet of fabric a grit or layer of abrasive particles, and a waterproof bond containing cellulosic material of a nature to maintain the bonding effect throughout the effective abrading life of the abrasive article when employed in a water abrading operation, and applying thereto a waterproof auxiliary coat containing cellulosic material.

75. The method of making a flexible abrasive article for use in a water abrading operation which includes applying to a flexible sheet of fabric a grit or layer of abrasive particles, and a waterproof bond containing cellulosic material and a modifying agent of a nature to maintain the bonding effect throughout the effective abrading life of the abrasive article when employed in a water abrading operation, and applying thereto a plurality of auxiliary coats.

80. The process of making a flexible waterproof abrasive article in the nature of sandpaper or the like which includes applying to a flexible sheet of fabric a grit or layer of abrasive particles, and a waterproof bond including modified cellulosic material of a nature to maintain the bonding effect throughout the effective abrading life of the abrasive article when employed in a water abrading operation, and applying an auxiliary coating to the article, said auxiliary coating including a modifying agent for reinforcing the bond.

85. A new article of manufacture in the nature of sandpaper including a flexible sheet of fabric, a grit or layer of abrasive particles, and a waterproof stable adhesive binder including cellulosic material interposed between the grit and said sheet and of a nature to maintain the bonding effect throughout the effective abrading life of the abrasive article when used in a water abrading operation, and an auxiliary coat applied to said article containing cellulosic material and a modifying agent for strengthening the bond.

90. As a new article of manufacture, sandpaper, including a flexible sheet of fabric as a base, a waterproof stable grit retaining adhesive including cellulosic material and a modifying agent applied to said fabric and adapted to form a connection with the base which is waterproof and stable when used in a water abrading operation but not detracting materially from the flexibility there-

70

75

80

85

90

95

100

105

110

115

120

125

130

- of when dry, and a pulverulent abrasive material applied to said adhesive.
19. As a new article of manufacture, sand paper, including a flexible sheet of material as a base, a waterproof stable grit retaining adhesive containing cellulosic material applied to said base and adapted to form a connection therewith which is waterproof and stable when used in a water abrading operation but not detracting materially from the flexibility thereof when dry, and a pulverulent abrasive material applied to said adhesive while still in a viscous state.
20. In a flexible and waterproof abrasive article, a flexible base, a flexible binder which includes cellulosic material and a modifying agent applied as a coating to said base united therewith to form a substantially homogeneous piece which is flexible, stable, waterproof and highly resistant to deterioration when used in a water abrading operation, and a pulverulent abrasive material carried by said binder.
21. In a flexible and waterproof abrasive article, a flexible base, a flexible binder which includes cellulosic material and a modifying agent applied as a coating to said base to partially solve the same and unite therewith to form a substantially homogeneous piece which is flexible, stable, waterproof and highly resistant to deterioration when used in a water abrading operation, and a pulverulent abrasive material carried by said binder.
22. An abrasive product comprising a flexible backing having abrasive grains attached thereto by a nitro-cellulose composition containing a resin.
23. An abrasive product comprising a flexible backing having abrasive grains attached thereto by a nitro-cellulose composition containing a resin and a plasticizer.
24. An abrasive product comprising a flexible backing having abrasive grains attached thereto by a nitro-cellulose composition, including an acetate, an alcohol, a ketone, benzol, a plasticizer, and a resin.
25. An abrasive product comprising a flexible backing having abrasive grains attached thereto by a nitro-cellulose binder containing an acetate, an alcohol, a ketone, benzol, camphor, and a resin.
26. An abrasive product comprising a flexible backing having abrasive grains attached thereto by a nitro-cellulose composition containing an acetate, an alcohol, a ketone, a benzol-type hydro-carbon, and a plasticizer.
27. An abrasive product comprising a flexible backing having abrasive grains attached thereto by a nitro-cellulose composition containing a solvent, camphor, and a resin.
28. An abrasive product comprising a flexible backing having abrasive grains attached thereto by a binding material containing nitro-cellulose, a resin, and a plasticizer.
29. An abrasive product comprising a flexible backing having abrasive grains attached thereto by a binder consisting of nitro-cellulose composition, a resin, and a camphor.
30. An abrasive product comprising a flexible backing having abrasive grains secured thereto by a composition containing nitro-cellulose, a high boiling solvent, a low boiling solvent, a plasticizer, and a resin.
31. An abrasive product comprising a flexible backing having abrasive grains attached thereto by a nitro-cellulose composition containing nitro-cellulose, a resin for giving body to nitro-cellulose, and a substance for rendering the composition tough and permanent and for overcoming the brittleness of the resin.
32. An abrasive product comprising a flexible backing having abrasive grains attached thereto by a flexible film containing nitro-cellulose, a resin for giving body to the nitro-cellulose, and a plasticizer for rendering the film flexible, tough and permanent.
33. An abrasive product comprising a flexible backing having abrasive grains attached thereto by a film which is resistant to water, such film being deposited from a slow evaporating nitro-cellulose composition in solution with a low boiling solvent, a high boiling solvent for retarding the evaporation thereof and by which an even spreading of the film is secured, a resin for giving body to the composition, benzol, which forms a solvent for the resin, and a plasticizer for imparting permanent toughness and flexibility to the film.
34. As a new article of manufacture a sandpaper product comprising a fabric base and abrasive material adhesively associated with said base by waterproof cellulosic coating material, said coating material containing a filler and also an emollient to maintain flexibility in the filler and the associated cellulosic material.
35. As a new article of manufacture a sandpaper product comprising a fabric base, abrasive material adhesively associated with said base, and a waterproof coating of cellulosic material, resin and oil, in which the cellulosic material maintains the position of the abrasive grains on the base, the resin serving as a filler and the oil as an emollient to maintain flexibility.
36. As a new article of manufacture, a sandpaper product comprising a fabric base and abrasive material adhesively associated with one surface of said base by waterproof coating material, the other surface of said base being covered with a cellulosic coating material containing a filler and also an emollient to maintain flexibility in the filler and the associated cellulosic material, said coating constituting a protective film to prevent frictional displacement of the fibres constituting the fabric base in the use of the article.
37. An article of manufacture such as set

forth in claim 36 in which the abrasive material and the coating material by which it is adhesively associated with the base adhesively supports an added coating of waterproof cellulosic material containing a filler and also an emollient to maintain flexibility in the filler and the associated cellulosic material forming a film in the nature of a matrix for the abrasive particles through which the abrasive particles, as they wear away, gradually penetrate without disturbing the matrix effect of said added film.

38. As a new article of manufacture, a sand-paper product comprising a fabric base and abrasive material adhesively associated with one surface of said base by waterproof coating material, the other surface of said base being covered with a cellulosic coating material containing a filler and also an emollient consisting of an oil to maintain flexibility in the filler and the associated cellulosic material, said coating constituting a protective film to prevent frictional displacement of the fibres constituting the fabric base in the use of the article.

39. An article of manufacture such as set forth in claim 38 in which the abrasive material and the coating material, by which it is adhesively associated with the base, adhesively supports an added coating of waterproof cellulosic material containing a filler and also an emollient consisting of an oil to maintain flexibility in the filler and the associated cellulosic material forming a film in the nature of a matrix for the abrasive particles through which the abrasive particles, as they wear away, gradually penetrate without disturbing the matrix effect of said added film.

40. As a new article of manufacture, a sand-paper product comprising a fabric base, abrasive material adhesively associated with the surface of said base by a matrix consisting of cellulosic material modified by the addition thereto of a resinous filler, an emollient consisting of an oil and an acetate and a plasticizer.

41. An article of manufacture such as set forth in claim 40, in which the opposite surface of the fabric base is treated with a waterproofing material to prevent the frictional displacement of fibres when the paper is used wet.

42. As a new article of manufacture a sand-paper product comprising a fabric base, abrasive material adhesively associated with the surface of said base by a matrix consisting of cellulosic material modified by the addition thereto of a resinous filler and an emollient consisting of an oil and an acetate.

In testimony whereof I have hereunto signed my name.

RICHARD PAUL CARLTON.